

## UNITED STATES PATENT OFFICE

2,487,190

## DIESEL FUEL OILS

Herschel G. Smith, Wallingford, Troy L. Cantrell, Lansdowne, and Mark L. Hill, Yeadon, Pa., assignors to Gulf Oil Corporation, Pittsburgh, Pa., a corporation of Pennsylvania

No Drawing. Application May 14, 1947,  
Serial No. 748,130

2 Claims. (Cl. 44—71)

1

This invention relates to improved Diesel fuel oils and more particularly to Diesel fuel oils which contain small amounts of addition agents which improve the performance characteristics of Diesel engines that burn said improved Diesel fuel oils.

Diesel engines are generally operated with fuel oils that have a boiling range above that of gasoline and below that of a motor lubricant. They may for instance have initial boiling points of about 400° F. and end boiling points of about 700° F. In the operation of Diesel engines with such petroleum fuel oils various difficulties arise. Often varnish or gum forms on the piston surfaces, cylinder walls, valves, and atomizing apparatus of Diesel engines operating on such fuel oils, and the piston rings stick. Gum formation on the close fitting pintle valve of the fuel injection equipment results in a rapid drop in power and fluctuating combustion pressure due to inconsistent fuel injection. After several days of operation on ordinary Diesel fuel oils, power output and engine efficiency decrease and there is a noticeable amount of knocking when the speed of the engine is increased. The engine must frequently be overhauled, cleaned and adjusted to restore its operating efficiency. Diesel fuel oils used in operating marine Diesel engines often become contaminated with water. As little as 0.1 per cent of water in a Diesel fuel oil can cause corrosion of fuel injectors so serious that the injectors must necessarily be replaced. With certain straight-run light Pennsylvania type fuel oils the wear on the injectors and plungers is sufficient to render them inaccurate after a few days operation thereby causing erratic engine performance. In particular, small and medium size Diesel engines which usually operate on rather light fuel oils operate with lessened efficiency because of insufficient lubrication and corrosion of parts. Corrosion, wear and gum formation on the high pressure injection pumps, interior cylinder surfaces and piston rings appear to be the major causes for the lessened efficiency with which Diesel engines perform when they are operated on ordinary Diesel fuel oils.

It is an object of this invention to manufacture fuel oils for Diesel engines which will improve the power output and performance characteristics of such engines. A further object is to produce Diesel fuel oils which will deposit very little varnish or gum on the engine parts. A still further object is to provide Diesel fuel oils which will not corrode engine parts if said oils become contaminated with water. Another

2

object is to provide Diesel fuel oils which will tend to lessen the wear on the engine parts. Other objects will appear hereinafter.

These objects are accomplished in accordance with the present invention by making improved Diesel fuel oils which contain a small proportion of aliphatic amine salts made from a long chain primary aliphatic amine having at least 10 carbon atoms and the mixture of fatty acids obtained by partially hydrolyzing, from 10 to 50 per cent by weight, a sulfurized sperm oil, and which also contains the mixture of alcohols obtained by said hydrolysis and unhydrolyzed sulfurized sperm oil, said aliphatic amine salts, mixture of alcohols and unhydrolyzed sulfurized sperm oil being present in sufficient quantities to retard corrosion, wear, gum formation and ring sticking in a Diesel engine burning said Diesel fuel.

More particularly, the addition agent used in 20 our improved Diesel fuel oils is prepared by first subjecting a sulfurized sperm oil to a partial hydrolysis, from 10 to 50 per cent by weight of the sperm oil being hydrolyzed. The product of the hydrolysis consists of a mixture of the sulfurized fatty acids of the sperm oil, the sulfurized fatty alcohols of the sperm oil, and unhydrolyzed sulfurized sperm oil. The entire mixture is then neutralized with a long chain primary aliphatic amine having at least 10 carbon atoms. As may 25 be seen, therefore, our addition agent is a mixture of aliphatic amine salts of the sulfurized sperm oil fatty acids, the sulfurized sperm oil alcohols and sulfurized sperm oil.

The sulfurized sperm oil employed in the preparation of our addition agent may be prepared by reacting sulfur with sperm oil as set forth in U. S. Patent 2,179,066 to Herschel G. Smith. Partial hydrolysis of the sulfurized sperm oil may be accomplished in any manner known to the art, such as by heating in the presence of water and a fat splitting agent such as sulfuric acid. As has been stated, the hydrolysis is partial and from 10 per cent to 50 per cent by weight of the sulfurized sperm oil is hydrolyzed or split into sulfurized sperm oil fatty acids and sulfurized sperm oil alcohols.

The aliphatic amine salts used in our improved Diesel fuel oils are made from primary aliphatic amines having at least 10 carbon atoms and the mixture of fatty acids obtained by hydrolyzing sulfurized sperm oil. The normal straight chain primary aliphatic amines used in preparing the amine salts used in the present invention preferably contain from 10 to 20 carbon atoms. Usually normal straight chain primary alkyl amines such

as decyl amine, undecyl amine, dodecyl amine, tetradecyl amine, cetyl amine, octadecyl amine and eicosyl amine are employed, but it is also permissible to use unsaturated straight chain primary aliphatic amines such as undecenyl amine and 9,10-octadecenyl amine (also called oleyl amine). Mixtures of the straight chain primary alkyl amines, such as cocoamine, are often used because of their relative cheapness. Cocoamine is a commercial mixture of higher alkyl amines prepared from coconut oil fatty acids. It contains a major amount of primary dodecyl amine, and typical samples thereof have been found to have average molecular weights ranging from 200 to 210.

The aliphatic amine salts used in our improved Diesel fuel oils are made by reacting approximately equimolecular proportions of amines, such as those mentioned in the preceding paragraph, with the mixture of fatty acids obtained by hydrolyzing sulfurized sperm oil. One of the amine salts which has been found to be a very desirable addition agent to Diesel fuel oils is the cocoamine salt of the mixture of fatty acids obtained by hydrolyzing sulfurized sperm oil.

The following examples further illustrate our invention:

*Example I.*—A sulfurized sperm oil was partially hydrolyzed to the extent of 10 per cent by weight, and the resulting partially hydrolyzed sulfurized sperm oil was neutralized with cocoamine. Ten parts by weight of the mixture of cocoamine salts of sulfurized sperm oil fatty acids, sulfurized sperm oil alcohols and unhydrolyzed sulfurized sperm oil were then blended with 90 parts by weight of a Texas oil having a viscosity of 1200 SUV at 100° F. to form a concentrate. The concentrate had the following properties:

|                 |      |      |
|-----------------|------|------|
| Gravity         | °API | 22.0 |
| Viscosity, SUV: |      |      |
| 100° F          |      | 1490 |
| 210° F          |      | 86   |
| Flash, OC       | °F   | 460  |
| Fire, OC        | °F   | 510  |
| Pour            | °F   | +5   |

*Example II.*—A sulfurized sperm oil was partially hydrolyzed to the extent of 50 per cent by weight, and the resulting partially hydrolyzed sulfurized sperm oil was neutralized with cocoamine. Ten parts by weight of the resulting mixture were then blended with 90 parts by weight of a Texas oil having a viscosity of 1200 SUV at 100° F. to form a concentrate. The concentrate had the following properties:

|                 |      |      |
|-----------------|------|------|
| Gravity         | °API | 21.8 |
| Viscosity, SUV: |      |      |
| 100° F          |      | 1492 |
| 210° F          |      | 86   |
| Flash, OC       | °F   | 465  |
| Fire, OC        | °F   | 515  |
| Pour            | °F   | +15  |

The above concentrates when added to a Diesel fuel oil markedly improved the performance characteristics of a Diesel engine burning said Diesel fuel oil. Generally, small amounts of our addition agents are sufficient to confer the desired improvement. Thus from 0.1 to 10.0 per cent by volume of the above concentrates, or from 0.01 to 1.0 per cent by weight of the addition agent per se, may be employed. In general, the addition agent is employed in amounts sufficient to retard corrosion, wear, ring sticking and gum formation in a Diesel engine burning said Diesel

fuel oil. Preferably 0.5 per cent by volume of the above concentrate, or 0.05 per cent by weight of the addition agent per se is employed. If desired we may dispense entirely with the formation of concentrates and add our addition agent directly to the Diesel fuel oil in the desired proportions.

*Example III.*—An improved light Diesel fuel was prepared by blending 0.5 per cent by volume of the concentrate prepared according to Example I and 99.5 per cent by volume of Diesel fuel oil. A comparison of the properties of the improved and unimproved fuel oils is as follows:

|                                               | Diesel<br>Fuel<br>Base Oil | Improved<br>Diesel<br>Fuel Oil |
|-----------------------------------------------|----------------------------|--------------------------------|
| Gravity, ° API                                | 42.5                       | 42.6                           |
| Viscosity, SUV, 100° F                        | 31                         | 31                             |
| Flash, P-M, ° F                               | 146                        | 146                            |
| Pour, ° F                                     | -60                        | -40                            |
| Sulfur, L, per cent                           | 0.05                       | 0.08                           |
| Carbon Residue, per cent                      | trace                      | trace                          |
| Carbon Residue on 10% Bottoms, per cent       | trace                      | trace                          |
| Corrosion Test No. 1 of Patent No. 2,371,883: |                            |                                |
| Steel Strip Appearance                        | rust                       | bright                         |
| Area Rusted, per cent                         | 100                        | nil                            |
| Neutralization No.                            | nil                        | nil                            |
| Acid Heat, ° F, ASTM D481-39                  | nil                        | nil                            |
| Aniline Point, ° F, ASTM D611-44T             | 145                        | 145                            |
| Diesel Index No.                              | 61.7                       | 61.7                           |
| Cetane No., ASTM D813-43T                     | 63                         | 63                             |
| Distillation, Gas Oil, ASTM D158-41:          |                            |                                |
| Over Point, ° F                               | 347                        | 347                            |
| End Point, ° F                                | 524                        | 530                            |
| 10% at ° F                                    | 386                        | 386                            |
| 50% at ° F                                    | 429                        | 432                            |
| 90% at ° F                                    | 488                        | 494                            |

*Example IV.*—A heavy Diesel fuel oil was prepared by blending 0.5 per cent by volume of the concentrate prepared according to Example II with 99.5 per cent by volume of a heavy Diesel fuel oil. A comparison by the properties of the improved and unimproved fuel oils is as follows:

|                                                     | Base<br>Oil | Improved<br>Oil |
|-----------------------------------------------------|-------------|-----------------|
| Gravity, ° API                                      | 24.5        | 24.4            |
| Viscosity, SUV:                                     |             |                 |
| 100° F                                              | 162         | 168             |
| 210° F                                              | 44          | 44              |
| Flash, P-M, ° F, ASTM D93-46                        | 250         | 250             |
| Pour, ° F                                           | +40         | +35             |
| Sulfur, L, per cent                                 | 0.40        | 0.45            |
| Water and Sediment, per cent                        | 0.10        | 0.10            |
| Sediment, per cent, ASTM D473-38T                   | 0.01        | 0.01            |
| Carbon Residue, per cent                            | 1.50        | 1.50            |
| Precipitation No.                                   | trace       | trace           |
| Ash, per cent                                       | 0.01        | 0.01            |
| BTU/lb, Gross                                       | 19,188      | 19,188          |
| Corrosion Test No. 1 of U. S. Patent No. 2,371,883: | rust        | bright          |
| Steel Strip Appearance                              | rust        | bright          |
| Area Rusted, per cent                               | 100         | nil             |

The Diesel fuel oils of the present invention such as those described in the preceding examples display many advantages over ordinary Diesel fuel oils. The close fitting pintle valves in the injection equipment of Diesel engines burning our improved fuel oils do not become covered with gum or corroded, and therefore the combustion pressure and power output remain constant even after more than 1000 hours of operation. This is an important advantage especially in connection with the operation of marine Diesel engines such as those used in power barges. Our new Diesel fuel oils substantially prevent corrosion and wear of the high pressure injection pumps, interior cylinder surfaces and piston rings, and reduce the tendency for piston rings to stick. Our Diesel fuels thus improve markedly the performance of Diesel engines, particularly

those of small and medium size that usually operate on rather light fuel oils. The Diesel oils of the present invention decrease the tendency toward ring sticking and varnish formation on cylinder walls, valves and atomizing apparatus, thereby improving engine performance, power output and engine efficiency. The speed of Diesel engines burning our improved fuel oils may be increased with less knocking, and such engines will operate for a longer running time without having to be overhauled. If our Diesel fuel oils become contaminated with a little water, no serious corrosion of the injectors will ensue, since the addition agents added to our fuel oils increase water tolerance. The wear on the plungers and injectors decreases considerably when our fuel oils are employed. Our improved Diesel fuel oils successfully counteract many of the factors that decrease the efficiency of Diesel engines operating on ordinary Diesel fuels.

We claim:

1. An improved Diesel fuel oil which consists of Diesel fuel oil and from about 0.01 per cent to about 1.0 per cent by weight of the products obtained by neutralizing with a long chain primary

15 aliphatic amine having at least 10 carbon atoms the mixture of fatty acids, alcohols and sulfurized sperm oil obtained by partially hydrolyzing, from 10 to 50 per cent by weight, a sulfurized sperm oil.

2. An improved Diesel fuel oil which consists of Diesel fuel oil and about 0.05 per cent by weight of the products obtained by neutralizing with cocaoamine the mixture of fatty acids, alcohols and sulfurized sperm oil obtained by partially hydrolyzing, from 10 to 50 per cent by weight, a sulfurized sperm oil.

10

15

HERSCHEL G. SMITH.  
TROY L. CANTRELL.  
MARK L. HILL.

#### REFERENCES CITED

The following references are of record in the file of this patent:

#### UNITED STATES PATENTS

| Number    | Name     | Date           |
|-----------|----------|----------------|
| 2,179,066 | Smith    | Nov. 7, 1939   |
| 2,330,524 | Shields  | Sept. 28, 1943 |
| 2,344,016 | Anderson | Mar. 14, 1944  |
| 2,401,993 | Wasson   | June 11, 1946  |

20

25